# EUROPEAN PATENT SPECIFICATION

(11) **EP 1 736 593 B1**
(45) Date of publication and mention of the grant of the patent: **24.11.2010**
(21) Application number: 06011813.0
(22) Date of filing: 08.06.2006
(51) Int. Cl.: D06N 3/00, D06N 3/14

(54) **Microfibrous non-woven chamois fabric having a high light fastness and process for its preparation**
Mikrofaseriges, wildlederartiges Vliesstoff mit einer hoher Lichtechtheit und Verfahren zu dessen Herstellung
Tissu microfibreux chamois de type nontissé ayant une grande solidité à la lumière et procédé de fabrication

(30) Priority: 24.06.2005 IT MI20051202
(43) Date of publication of application: 27.12.2006
(73) Proprietor: ALCANTARA S.p.A., 20138 Milano (IT)
(72) Inventor: Bianco, Paola, 05022 Amelia (TR) (IT); Giancarlini, Luca, 05100 Terni (IT); Hashimoto, Takafumi, Shiga (JP)
(74) Representative: Bottero, Carlo

(56) References cited:
- EP-A- 0 964 096
- EP-A1- 0 557 247
- IT-B- 1 196 456
- "34. Chemiefasertagung Dornbirn" 1995, OESTERREICHISCHES CHEMIEFASER-INSTITUT , WIEN (AT) , XP009089884 "Printing on Automotive Textiles (PES). A new technology in the Automotive industry." by J. Kath, P. Haerri, P. Johnson, J. McGarrie, R. Rommel.
- "UTILISATION DES ABSORBEUR D'U.V. POUR MINIMISER LA DEGRADATION PHOTOCHIMIQUE DES COLORANTS DISPERSES ET DES FIBRES DE POLYESTER" L'INDUSTRIE TEXTILE, no. 1257, 1 September 1994 (1994-09-01), page 96, XP000507430 Paris (FR) ISSN: 0018-8689
- W. WANG, A. TANIGUCHI, M. FUKUHARA, T. OKADA: JOURNAL OF APPLIED POLYMER SCIENCE, vol. 74, 1999, pages 306-310, XP002452286
- P. RYS & H. ZOLLINGER: "Farbstoffchemie: ein Leitfaden" 1982, VERLAG CHEMIE , WEINHEIM , XP002452291 * page 7 - page 11 *
- "SAE J1885: Accelerated Exposure of Automotive Interior Trim Components Using a Controlled Irradiance Water Cooled Xenon-Arc Apparatus" , XP009125444

## Description

The present invention relates to a microfibrous non-woven chamois fabric (hereinafter also microfibrous non-woven fabric) having a high light fastness. More specifically, the high level of colour fastness to light is obtained by using one or more UV stabilizers selected from benzotriazoles, triazines and benzophenones, at least one of the components belonging to the group of triazines.

It is known that the light fastness of microfibrous non-woven fabrics is generally not completely satisfactory for various particular applications, for example car upholstery. Attempts have been made in the past to enhance light fastness. For example the patent IT 1196456 describes the production of a microfibrous non-woven fabric prepared by using at least one UV stabilizer, selected from benzophenones and benzotriazoles, in the dyeing phase. This technology, however, has various limitations as its efficacy is limited to certain wave-lengths.

A microfibrous non-woven chamois fabric has now been found, which overcomes the drawbacks mentioned above as it has a high light fastness in the UV region.

In accordance with this, the present invention relates to a microfibrous non-woven according to claim 1.

According to the invention, the composition of UV stabilizers consists of:
(i) triazine and derivatives thereof
(ii) benzophenones and benzotriazoles and relative blends;
the weight % of compound (i) with respect to the sum of (i) + (ii) preferably being at least 30%.

Typical examples of benzophenone derivatives are: 2,4-dihydroxybenzophenone, 2-hydroxy-4-methoxybenzophenone,
2-hydroxy-4-octyloxybenzophenone, 2-hydroxy-4-isooctyloxy benzophenone, 2-hydroxy-4-dodecyloxy benzophenone, 2,2'-dihydroxy-4-methoxybenzophenone, 2,2',4,4'-tetrahydroxy benzophenone, 2,2-dihydroxy-4,4'-dimethoxybenzophenone, 2-hydroxy-4-methoxy-5-solfobenzophenone, 2-hydroxy-4-benzyloxybenzophenone.

Typical examples of benzotriazole derivatives are:
2-(2'hydroxyphenyl) benzotriazole, 2-(2'hydroxy-5-methylphenyl) benzotriazole, 2-(2'-hydroxy-3',5'-di-t-butylphenyl)-5-chlorobenzotriazole, 2-(2'-hydroxy-3'sec-butyl-5'-methylphenyl) benzotriazole, 2-(2'-hydroxy-5'-octylphenyl) benzotriazole, 2-[2'-hydroxy-3',5'-(di-t-butyl) phenyl] benzotriazole, 2-[2'-hydroxy-3',5'-(di-t-amyl)phenyl] benzotriazole, 2-[2'-hydroxy-3',5'-di-(α,α--dimethylbenzyl)phenyl] benzotriazole, 2-(3'-t-butyl-2'-hydroxy-5'-methylphenyl)-5'-chlorobenzotriazole, 2-(2'-hydroxy-3',5'-di-t-butyl)-5-chlorobenzotriazole, 2-(2'-hydroxy-5'-(1,1,3,3-tetramethylbutyl)phenyl) benzotriazole, 2-(2'-hydroxy-4'-octyloxyphenyl) benzotriazole, 2-(2'-hydroxy-3',5'-di-t-amyl-phenyl) benzotriazole.

Typical examples of triazine derivatives are:
2,4,6(triphenyl)-1,3,5-triazine, 2,4,6-tri(2-hydroxy-4-octyloxyphenyl)-1,3,5-triazine, 2(2-hydroxy-4-hcxyloxy-phenyl)-4,6-bisphenyl)-1,3,5-triazine, 2(2-hydroxy-4-octyloxyphenyl)-4,6-bis(2,4-dimethylphenyl)-1,3,5-triazi-ne, 2-(2,4-dihydroxyphenyl)-4,6-bis(2,4-dimethylphenyl)-1,3,5-triazine,2,4-bis(2-hydroxy-4-propyl-oxyphenyl)-6-(2,4-dimethylphenyl)-1,3,5-triazine, 2-(2-hydroxy-4-octyloxyphenyl)-4,6-bis(4-methylphenyl)-1,3,5-triazine, 2-(2-hydroxy-4-dodecyloxyphenyl)-4,6-bis(2,4-dimethylphenyl)-1,3,5-triazine, 2-(2-hydroxy-4-tridecyloxyphenyl)-4,6-bis (2,4-dimethylphenyl)-1,3,5-triazine, 2-[2-hydroxy-4-(2-hydroxy-3-butyloxypropanyloxy)-phenyl]-4,6-bis(2,4-dimethyl)-1,3,5-triazine, 2-[2-hydroxy-4-(2-hydroxy-3-octyloxy propyloxyoctyloxypropyloxy)-phenyl]-4,6-bis(2,4-dimethyl)-1,3,5-iriazine, 2-[4-(dodecyloxy/tridecyloxy-2-hydroxypropoxy)-2-hydroxyphenyl]4,6-bis(2,4-dimethylphenyl) -1,3,5-triazine, 2-[2-hydroxy-4-(2-hydroxy-3-dodecyloxypropoxy)-phenyl]-4,6-bis(2,4-dimethyl-phenyl)-1,3,5-triazine, 2-(2-hydroxy-4-hexyloxy)phcnyl-4,6-diphenyl-1,3,5-triazine, 2-(2-hydroxy-4-methoxyphenyl)-4,6-diphenyl-1,3,5-triazine, 2,4,6-tris[2-hydroxy-4-(3-butoxy-2-hydroxypropoxy)phenyl]-1,3,5-triazine, 2-(2-hydroxy-phenyl)-4-(4-methoxyphenyl)-6-phenyl-1,3 ,5-triazine, 2-{2-hydroxy-4-[3-(2-ethylhexyl-1-oxy)-2-hydroxypropyloxy-phenyl}-4,6-bis-(2,4-dimethylphenyl)-1,3,5-triazine.

The non-woven fabric of the present invention shows a light fastness value higher than 3 (for details sec the experimental part).

If microfibres consisting of polyethylene terephthalate alone are used, the product of the present invention has, upon reflectance spectrophotometric analysis in the colour space of CIELAB (1976), a luminosity value L lower than 35 (with a D65 illuminator and an observation angle of 10°). This L value proved to be equal to 32 in the material described in the experimental part.

If microfibres consisting of polyethylene terephthalate and polyethylene terephthalate dyeable with cationic dyes are used, the product of the present invention has, upon reflectance spectrophotometric analysis in the colour space of CIELAB (1976), a luminosity value L ranging from 45 to 75 (with a D65 illuminator and an observation angle of 10°). This L value proved to be equal to 55 in the material described in the experimental part.

The present invention also relates to a process for the preparation of microfibrous non-woven chamois fabric comprising the following steps:
(y1) preparation of unbleached, microfibrous non-woven chamois fabric;
(y2) dyeing of the unbleached fabric obtained in step (y1);
(y3) treatment of the dyed product obtained at the end of step (y2) with a composition of UV stabilizers, of which at least one has a maximum absorption at wave-lengths ranging from 270 to 285 nm.

Steps (y2) - (y3) can be carried out in the above sequence or simultaneously.

The preparation of unbleached, microfibrous non-woven chamois fabric (step y1) is effected using techniques well- known to experts in the field, for example according to what is described in EP-A-0584511, US-A-3,716,614 and US-A-3,531,368, EP-A-20030028443 and in the Italian patent ITMI20022685A, all in the name of the Applicant. These patents are therefore mentioned as representing an integrant base of this description for any reference of interest. More specifically, a fiber is first prepared in staple form, consisting of polyethylene terephthalate, polyethylene terephthalate dyeable with cationic dyes or polytrimethylene terephthalate microfibres, etc.. having a denier value ranging from 0.011 to 0.44 dtex (0.01 to 0.4 deniers), preferably in the range of 0.089 to 0.167 dtex (0.08÷0.15 deniers), in a polystyrene matrix or a styrene copolymer or co-polyestcr or polyvinyl alcohol, etc.. which acts as a "sheath". Generally the fiber in staple form has the following characteristics: from 1.56 to 11.1 dtex (1.4 to 10 deniers) and preferably from 2.78 to 6.67 dtex (2.5 to 6 deniers); length from 30 to 150 mm preferably in the range of 30÷100 mm; draw ratio from 2/1 to 5/1; curlings from 4 to 15 per centimetre. The fiber in staple form can also contain 30÷90 parts by weight of polyethylene terephthalate, polyethylene terephthalate dyeable with cationic dyes or polytrimethylene terephthalate microfibres, etc.., 10÷70 parts by weight of polystyrene matrix or a styrene copolymer or a co-polyester or polyvinyl alcohol, etc.. and possibly different types of additives.

An unbleached felt is prepared with one or more of said fibres in staple form, which undergoes needl ing to form a needled felt having a suitable density in the order of 0.15÷0.35 g/cm³. The needled felt is then immersed in an aqueous solution of polyvinyl alcohol, for example from 10 to 30% by weight, and, after drying, is immersed in a solvent capable of completely solubilizing the matrix. The resulting product is dried and represents the non-woven fabric of microfibres, to which an elastomeric matrix, preferably polyurethane, is applied, by immersion in a solution/dispersion.

The term polyurethane refers to a polymer consisting of flexible segments (soft segments) and rigid segments (hard segments).

The flexible segments can be polymeric chains based on the following polymers and/or copolymers and/or blends thereof, having a weight average molecular weight ranging from 500÷5,000, preferably from 600 to 2,000:
- polyethers, such as, for example, derivatives of polytetramethylene glycol diol (PTMG), polyethylene glycol diol (PEG), polypropylene glycol diol (PPG);
- polyesters, such as, for example, esters of adipic acid such as polyhexamethylene adipate diol (PHA), poly(3-methyl pentamethylene) adipate diol (PMPA) or polyneopentyl adipate diol (PNA); other polyesters can be produced by the opening of cyclic molecules, such as caprolactone (thus obtaining caprolactone diol, in short PCL);
- polycarbonates, such as , for example, polyhexamethylene carbonate diol (PHC), polypentamethylene carbonate diol (PPMC), poly-(3-methyl-pentamethylene carbonate) diol(PMPC), polytetramethylene carbonate diol (PTMC), blends thereof and copolymers.

Polyesters formed by the copolymerization of the polyethers and polyesters mentioned above, can be used as flexible segments, as well as polyester-co-polycarbonates obtained by the copolymerization of polyesters and polycarbonates.

The polymers of the polyester, polycarbonate type and co-polymers of the polyester-polycarbonate type and of the polyester-polyether type having a number average molecular weight ranging from 500 to 5,000, preferably from 600 to 2000, containing groups of a hydrophilic nature, and/or with a negative charge, such as, for example, dimethyl propionic acid (DMPA) or functionalized sulphonic acids, can also be used as flexible segments; polyurethane dispersions can be obtained in this way.

The rigid segments refer to portions of the polymeric chains obtained from the reaction of an aromatic diisocyanate, such as, for example, methylene-bis-(4-phenylisocyanate) (MDI) or toluene diisocyanate (TDI) or an aliphatic or cyclo-aliphatic diisocyanate with a diamine or glycolic chain. It is well-known, in fact, that the completion of the polyurethane synthesis can be effected with diamines, thus obtaining polyurethane-ureas, or with glycols obtaining polyurethane.

Possible diamines which can be used as chain extenders in the production of polyurethane-ureas are, among aliphatic products, ethylene diamine (EDA), 1,3-cyclohexane diamine (1,3-CHDA), 1,4-cyclohexane diamine (1,4-CHDA) isophorondiamine (IPDA), 1,3-propylene diamine (1,3-PDA), and relative blends. Typical examples of aromatic diamines to be used as chain extenders are 3,3'-dichloro-4,4'-diamine diphenyl methane, methylene-bis(4-phenylamine) (MPA), 2,4-diamino-3,5-diethyltoluene, 2,4-diamino-3,5-di(methylthio) toluene. The above aliphatic and/or aromatic diamines can be added as such or developed in situ by reaction between the corresponding isocyanate and water. The chain extension in the polyurethane in the true sense, can also be obtained with diols such as ethylene glycol, tetramethylene glycol and relative blends. The chain extension can also be obtained through dicarboxylic acids such as malonic, succinic, adipic acids.

The above preparations of the various polyurethanes are well-known to experts in the field.

Returning to step (y1), if polymeric solutions are used, the impregnated product is squeezed through two rolls and coagulation in water is effected, for example at 20÷50°C. A coagulated sheet is obtained which is poured into hot water, for example at about 80°C, to extract the residual solvent and polyvinyl alcohol.

In the case of polymeric dispersions, the impregnated product is squeezed through two rolls, vapour coagulation is then effected, either in an acidic aqueous solution or in dry heat.

The coagulated sheet is then dried, cut into sheets of 0.6÷1.5 mm which are subjected to polishing to raise the surface pile.

The unbleached synthetic composite microfibrous non-woven fabric thus obtained at the end of the step (y1), is subjected to combined treatment of dyeing and contact with the UV stabilizer composition described above (steps y2 and y3 together) or, as an alternative, the fabric is first dyed (step y2) and then immersed (step y3) in an aqueous bath containing the UV stabilizers.

The whole material is then subjected to drying and thermo-setting.

As already mentioned, the present invention relates to the application of UV stabilizers according to the method described hereunder:
(i) Introduction of one or more UV stabilizers during the dyeing step. According to an embodiment of the present invention, the dyeing treatment and introduction of stabilizers is carried out in "circular" dyeing equipment, equipped with a Venturi nozzle, for example the equipment supplied by the company Hisaka Works Ltd.
   The dyeing cycle consists of a first dyeing step, in which the unbleached synthetic composite microfibrous non-woven fabric is put in contact with a mixture of dyes, one or more UV stabilizers selected from benzotriazoles, triazines and benzophenones in which at least one of the components belongs to the group of triazines, surface-active agents which disperse the dye and facilitate the passage to the fibre, pH conditions suitable for allowing the dye to penetrate inside the fibre, and dyeing auxiliaries. The maximum dyeing temperature, normally ranging from 10 to 140°C, is selected so as to bring the polymers forming the microfibre above their glass transition temperature, thus facilitating the diffusion of the dye and stabilizers in its interior.
   If microfibres of polyethylene terephthalate and/or polytrimethylene terephthalate, etc.. are used, the dyeing blend consists of dispersed dyes, preferably selected from the dispersed dyes of a non-azo type, whereas, when a microfibre of polyethylene terephthalate dyeable with cationic dyes is used, the dye blend consists of cationic dyes. If a mix of fibres consisting of polyethylene terephthalate and/or polytrimethylene terephthalate and polyethylene terephthalate dyeable with cationic dyes, is used, the blend of dyes consists of dispersed dyes and cationic dyes.
   The quantity of triazine dye used alone or in a blend with benzotriazole and/or benzophenone stabilizers, is suitably maintained with percentages of active principle ranging from 0.1 to 5% by weight with respect to the microfibrous non-woven fabric. Stabilizers can be added directly to the dyeing bath, or, preferably, pre-dispersed in a liquid vehicle containing from 10 to 40% by weight of active substance.
   In practice, the microfibrous non-woven fabric is circulated inside the dyeing equipment for 1 hour or so, at the highest dyeing temperature and, subsequently, subjected to cleaning treatment with sodium hydrosulphite in a basic environment.
   In addition to the dyeing treatment, it is possible to effect finishing treatment to confer other specific properties to the product, such as a softer feel. It is also possible to process the end product under heat, up to 250°C, for an amount of time strictly necessary for effecting, for example, coupling to other substrates, printing, embossing, lamination, injection printing, thermosetting.
(ii) Introduction of UV stabilizers after dyeing by padding; according to the process of the present invention, the introduction of one or more stabilizers selected from triazines, benzotriazoles, and benzophenones, at least one of the components belonging to the group of triazines is carried out on a microfibrous non-woven fabric dyed by immersion at room temperature in an aqueous solution containing the above stabilizers in a weight percentage ranging from 0.01 to 25%, different kinds of additives, pH regulators, bactericides, fungicides, etc...

The squeezing level adopted is between 20 and 70%. After removal of the aqueous solution, the material is dried at a temperature of 95 - 180°C preferably at about 140°C. The product thus obtained has excellent characteristics with respect to appearance, feel, lightness, velour and absence of tone differences between velour and background. More than anything else, the material obtained has a particularly high light resistance with respect to similar products of the known art, so that, for example, after exposure to the methods DIN 75 202 (3 fakra), D 47 1431 (150 hours), SAEJ 1885 225.6 KJ/m², the colour difference is not less than 3/4 of the grey scale. This characteristic makes the material particularly suitable for applications in the car industry, as car upholstery or similar uses. The evaluation of the colour fastness to light is effected by evaluating the colour variation before and after exposure, using the grey scale ISO 105A02. In the light exposure methods, the irradiating spectrum can also include radiations having wave-lengths of 270 to 700 nm; as known, UV radiations having a wave-length of 270 and 400 nm prove to be the most dangerous for colour fastness to light.

The following experimental examples are illustrative and non-limiting of the scope of the present invention:

### EXAMPLES

The following UV resistant products were used both singly and in a combination thereof:
1- Triazine derivative (produced by Ciba and called Cibafast^{®} P) : λₘₐₓ = 275 nm.
2- Benzotriazole derivative (produced by Ciba and called Cibafast^{®} PEX) : λₘₐₓ = 352 nm.
3- Benzophenone derivative (produced by Clariant and called Fadex^{®} ECS) : λₘₐₓ = 288 nm.

Examples 1 to 9 refer to the treatment of a microfibrous non-woven fabric consisting of PET alone; whereas examples 10 to 14 refer to the treatment of a microfibrous non-woven fabric consisting of blends of polyethylene terephthalate and polyethylene terephthalate dyeable with cationic dyes.

### Example 1 - PET microfibrous non-woven fabric without UV stabilizers

A fibre in staple form is prepared, made of polyethylene terephthalate microfibres 0.11 to 0.12 dtex (0.10÷0.11 deniers) in a polystyrene matrix, having the following characteristics: 4.22 dtex (3.8 deniers), length 51 mm, 5 curlings/cm, draw ratio 2.5/1. In particular, the fibre is made up of 57 parts by weight of polyethylene terephthalate microfibre, 43 parts by weight of polystyrene matrix. In a sectional view, the fibre reveals the presence of 16 microfibres of polyethylene terephthalate englobed in the polystyrene matrix. An unbleached felt is prepared with the fibre in staple form, subjected to needling to form a needled felt having a density of 0.185 g/cm³. The needled felt is immersed in a 20% by weight aqueous solution of polyvinyl alcohol and is then subjected to drying. The needled felt thus treated is subsequently immersed in trichloroethylene until complete dissolution of the polystyrene matrix of the fibres, with the consequent formation of a non-woven fabric of polyethylene terephthalate microfibres. The non-woven fabric produced is then dried and an intermediate product called felt is obtained.

The felt is immersed in the polyurethane elastomeric solution and the non-woven fabric thus impregnated is first squeezed by passing it through a pair of rolls and subsequently immersed for 1 hour in a water bath maintaining the temperature at 40°C. A coagulated sheet is thus obtained which is passed into a water bath heated to 80°C, to extract the residual solvent and polyvinyl alcohol. After drying, a composite microfibrous sheet is obtained which is cut into sheets having a thickness of 1 mm, which are subjected to polishing to raise the surface pile. A synthetic unbleached non-woven fabric is obtained having a thickness of 0.8 mm, which is subjected to dyeing in "JET" equipment, equipped with a "Venturi tube". In particular, the synthetic unbleached non-woven fabric is passed through the "Venturi tube" for 1 hour, at 125°C, in an aqueous dyeing bath containing the following dispersed dyes:
- dispersed Red dye (anthraquinone type) 2.5% by weight
- dispersed Blue dye (anthraquinone type) 28% by weight
- dispersed Orange dye (amino-ketone type) 10% by weight

After dyeing, a dyed microfibrous non-woven fabric is obtained which, after further treatment under reducing conditions with sodium hydrosulphite in an alkaline environment to eliminate the excess dye, is subjected to evaluation tests of the colour resistance to dry and wet rubbing (AATCC 8-2001), to soap washing (AATCC 61-2001), to dry washing and to light (SAEJ 1885 - 225 KJ/m²).

The evaluations, shown in the following table, relating to the dyed microfibrous non-woven fabric, were effected as follows:
a) as far as the colour discharge on a test sample is concerned (multifibre felt for washings and cloth for the rubbing) the soiling is evaluated by comparison with the grey scale ISO 105A03;
b) as far as the shade exchange of the sample, before and after the test, is concerned, the grey scale ISO 105A02 is used.

The evaluation is effected by comparing the shade exchange or dirt level with the codified contrasts by means of the appropriate grey scale; an evaluation of 5 corresponds to no change in shade/colour transfer, whereas a value of 1 corresponds to the maximum contrast on the grey scale used.

| TEST | Evaluation |
|---|---|
| Wet rubbing AATCC 8-2001 (colour discharge) | 4 |
| Dry rubbihn AATCC 8-2001 (colour discharge) | 4/5 |
| Washing with soap AATCC 61-2001 (colour change) | 5 |
| Washing with soap AATCC 69-2001 (color discharge) | 4/5 |
| Dry washing (shade exchange). | 5 |
| Dry washing (colour discharge) | 4/5 |
| Light fastness, SAE J 1885 225 KJ/m² (shade change) | 2/3 |

### Example 2 - 2% Benzotriazole

The same procedure is adopted as in example 1, adding a substituted benzotriazole to the dyeing bath, known in the market as Cibafast^{®} PEX of the company Ciba, in an active principle percentage of 2% by weight with respect to the microfibrous non-woven fabric. This additive is added to the dyeing bath pre-dispersed in a liquid vehicle.

A dyed, microfibrous non-woven fabric is obtained having a light fastness value of 3, determined as described in example 1 and with the other characteristics similar to those in said example 1.

### Example 3 - 2% Benzophenone

The same procedure is adopted as in example 1, adding a substituted benzophenone to the dyeing bath, known on the market as Fadex^{®} ECS of the company Clariant, in an active principle percentage of 2% by weight with respect to the microfibrous non-woven fabric. This additive is added to the dyeing bath pre-dispersed in a liquid vehicle.

A dyed, microfibrous non-woven fabric is obtained having a light fastness value of 3, determined as described in example 1 and with the other characteristics similar to those in said example 1.

### Example 4-2% Triazine

The same procedure is adopted as in example 1, adding a substituted triazine to the dyeing bath, known on the market as Cibafast^{®} P of the company Ciba, in an active principle percentage of 2% by weight with respect to the microfibrous non-woven fabric. This additive is added to the dyeing bath pre-dispersed in a liquid vehicle.

A dyed, microfibrous non-woven fabric is obtained having a light fastness value of 3/4, determined as described in example 1 and with the other characteristics similar to those in said example 1.

### Example 5 - 1% Benzotriazole and 1% Benzophenone

The same procedure is adopted as in example 1, adding a blend of UV stabilizers to the dyeing bath, consisting of Cibafast^{®} PEX in an active principle percentage of 1% by weight with respect to the microfibrous non-woven fabric, and Fadex^{®} ECS in an active principle percentage of 1 % by weight with respect to the microfibrous non-woven fabric. These additives are added to the dyeing bath pre-dispersed in a liquid vehicle.

A dyed, microfibrous non-woven fabric is obtained having a light fastness value of 3, determined as described in example 1 and with the other characteristics similar to those in said example 1.

### Example 6 - 1% Triazine and 1% Benzophenone

The same procedure is adopted as in example 1, adding a blend of UV stabilizers to the dyeing bath, consisting of Cibafast^{®} P in an active principle percentage of 1% by weight with respect to the microfibrous non-woven fabric, and Fadex^{®} ECS in an active principle percentage of 1% by weight with respect to the microfibrous non-woven fabric. These additives are added to the dyeing bath pre-dispersed in a liquid vehicle.

A dyed, microfibrous non-woven fabric is obtained having a light fastness value of 3/4, determined as described in example 1 and with the other characteristics similar to those in said example 1.

### Example 7 - 1% Triazine and 1% Benzotriazole

The same procedure is adopted as in example 1, adding a blend of UV stabilizers to the dyeing bath, consisting of Cibafast^{®} P in an active principle percentage of 1% by weight with respect to the microfibrous non-woven fabric, and Cibafast^{®} PEX in an active principle percentage of 1% by weight with respect to the microfibrous non-woven fabric. These additives are added to the dyeing bath pre-dispersed in a liquid vehicle. A dyed, microfibrous non-woven fabric is obtained having a light fastness value of 3/4, determined as described in example 1 and with the other characteristics similar to those in said example 1.

### Example 8 - 0.66% Triazine, 0.66% Benzotriazole and 0.66% Benzophenone

The same procedure is adopted as in example 1, adding a blend of UV stabilizers to the dyeing bath, consisting of Cibafast^{®} P in an active principle percentage of 0.66% by weight with respect to the microfibrous non-woven fabric, Cibafast^{®} PEX in an active principle percentage of 0.66% by weight with respect to the microfibrous non-woven fabric, and Fadex^{®} ECS in an active principle percentage of 0.66% by weight with respect to the microfibrous non-woven fabric. These additives are added to the dyeing bath pre-dispersed in a liquid vehicle.

A dyed, microfibrous non-woven fabric is obtained having a light fastness value of 4, determined as described in example 1 and with the other characteristics similar to those in said example 1.

### Example 9-1% Triazine, 1% Benzotriazole and 1% Benzophenone by padding

The same procedure is adopted as in example 1, but the already dyed microfibrous non-woven fabric is treated by dipping it into an aqueous solution (padding treatment) containing:
- substituted triazine commercially known as Cibafast^{®} P in an active principle percentage of 1% by weight;
- substituted benzotriazole commercially known as Cibafast^{®} PEX in an active principle percentage of 1% by weight;
- substituted benzophenone commercially known as Fadex^{®} ECS in an active principle percentage of 1% by weight.

The retention level adopted on the wet product was 117%. After removal from the water solution, the material is dried at a temperature of 100°C for about 3 minutes.

A dyed, microfibrous non-woven fabric is obtained having a light fastness value of 4, determined as described in example 1 and with the other characteristics similar to those in said example 1.

## Claims

1. A microfibrous non-woven chamois fabric, comprising:
microfibres selected from polyester microfibres;
an elastomeric matrix; and
a composition of UV stabilizers consisting of:
at least one triazine or derivatives thereof, having a maximum absorbance at wavelengths ranging from 270 to 285 nm; and
at least one compound selected from benzophenones, benzotriazoles and blends thereof.

2. The non-woven fabric according to claim 1, wherein the elastomeric matrix is selected from polyurethane, urea-polyurethane, and blends thereof.

3. The non-woven fabric according to claim 1, wherein the polyester is selected from polyethylene terephthalate, polymethylene terephthalate, polyethylene terephthalate dyeable with cationic dyes, and blends thereof.

4. The non-woven fabric according to claim 1, wherein the polyester is dyed with a mix of dispersed dyes, at least one of the dispersed dyes comprising a dispersed anthraquinone dye.

5. The non-woven fabric according to claim 1, wherein the at least one triazine or derivatives thereof is present in the composition of UV stabilizers in an amount of at least 30% by weight.

6. The non-woven fabric according to claim 9, wherein the composition of UV stabilizers is present in an amount of 0.5 to 5% by weight with respect to the microfibrous non-woven fabric.

7. The non-woven fabric according to claim 6, wherein the composition of UV stabilizers is present in an amount of 1.5 to 3% by weight with respect to the microfibrous non-woven fabric.

8. The non-woven fabric according to claim 3, wherein the polyester is polyethylene terephthalate.

9. The non-woven fabric according to claim 3, wherein the polyester consists of a blend of polyethylene terephthalate, and polyethylene terephthalate dyeable with cationic dyes.

10. A process for the preparation of the microfibrous non-woven chamois fabric of claim 1, the process comprising:
preparing an unbleached microfibrous non-woven chamois fabric;
dyeing the unbleached microfibrous non-woven chamois fabric to obtain a dyed product; and
treating the dyed product with a composition of UV stabilizers consisting of:
at least one triazine or derivatives thereof, having a maximum absorption at wavelengths from 270 to 285 nm; and
at least one compound selected from benzophenones, benzotriazoles and blends thereof.

11. The process according to claim 10, wherein the dying and treating steps are effected contemporaneously.

## Patentansprüche

1. Mikrofaseriger, wildlederartiger Vliesstoff, umfassend:
aus Polyestermikrofasern ausgewählte Mikrofasern;
eine Elastomer-Matrix; und
eine Zusammensetzung von UV-Stabilisatoren, bestehend aus:
mindestens einem Triazin oder Derivaten davon, mit einem Absorptionsmaximum bei einem Wellenlängenbereich von 270 bis 285 nm; und
mindestens einer aus Benzophenonen, Benzotriazolen und Mischungen davon ausgewählten Verbindung.

2. Vliesstoff nach Anspruch 1, wobei die Elastomer-Matrix aus Polyurethan, Harnstoff-Polyurethan und Mischungen davon ausgewählt ist.

3. Vliesstoff nach Anspruch 1, wobei das Polyester aus Polyethylenterephthalat, Polymethylenterephthalat, mit kationischen Farbstoffen färbbarem Polyethylenterephthalat und Mischungen davon ausgewählt ist.

4. Vliesstoff nach Anspruch 1, wobei das Polyester mit einem Gemisch aus dispergierten Farbstoffen gefärbt ist, wobei mindestens eines der dispergierten Farbstoffe einen Anthrachinon-Dispersionsfarbstoff umfasst.

5. Vliesstoff nach Anspruch 1, wobei das mindestens eine Triazin oder Derivate davon in der Zusammensetzung von UV-Stabilisatoren in einer Menge von mindestens 30 Gew.-% vorhanden sind.

6. Vliesstoff nach Anspruch 1, wobei die Zusammensetzung von UV-Stabilisatoren in einer Menge von 0,5 bis 5 Gew.-% bezogen auf den mikrofaserigen Vliesstoff vorhanden ist.

7. Vliesstoff nach Anspruch 6, wobei die Zusammensetzung von UV-Stabilisatoren in einer Menge von 1,5 bis 3 Gew.-% bezogen auf den mikrofaserigen Vliesstoff vorhanden ist.

8. Vliesstoff nach Anspruch 3, wobei das Polyester Polyethylenterephthalat ist.

9. Vliesstoff nach Anspruch 3, wobei das Polyester aus einer Mischung aus Polyethylenterephthalat und mit kationischen Farbstoffen färbbarem Polyethylenterephthalat besteht.

10. Verfahren zur Herstellung des mikrofaserigen, wildlederartigen Vliesstoffes nach Anspruch 1, umfassend:
Herstellen eines ungebleichten, mikrofaserigen, wildlederartigen Vliesstoffes;
Färben des ungebleichten, mikrofaserigen, wildlederartigen Vliesstoffes zum Erhalten eines gefärbten Erzeugnisses; und
Behandeln des gefärbten Erzeugnisses mit einer Zusammensetzung von UV-Stabilisatoren, bestehend aus:
mindestens einem Triazin oder Derivaten davon, mit einem Absorptionsmaximum bei einem Wellenlängenbereich von 270 bis 285 nm; und
mindestens einer aus Benzophenonen, Benzotriazolen und Mischungen davon ausgewählten Verbindung.

11. Verfahren nach Anspruch 10, wobei die Schritte des Färbens und Behandelns gleichzeitig durchgeführt werden.

## Revendications

1. Tissu microfibreux chamois de type non tissé, comprenant :
une matrice élastomère ; et
une composition de stabilisateurs UV incluant :
au moins une triazine ou ses dérivés, ayant une absorbance maximale à des longueurs d'onde allant de 270 à 285 nm ; et
au moins un composé sélectionné à partir de benzophénones, de benzotriazoles, et des mélanges de ceux-ci.

2. Tissu de type non tissé selon la revendication 1, dans lequel la matrice élastomère est sélectionnée à partir de polyuréthane, de polyuréthane-urée, et des mélanges de ceux-ci.

3. Tissu de type non tissé selon la revendication 1, dans lequel le polyester est sélectionné à partir de polyéthylène-téréphtalate, de polyméthylène-téréphtalate, de polyéthylène-téréphtalate colorable avec des colorantes cationiques, et des mélanges de ceux-ci.

4. Tissu de type non tissé selon la revendication 1, dans lequel le polyester est coloré avec un mélange de colorants dispersés, au moins l'un des colorants dispersés comprenant un colorant anthraquinonique dispersé.

5. Tissu de type non tissé selon la revendication 1, dans lequel ladite triazine ou ses dérivés sont présents dans la composition des stabilisateurs UV à hauteur de 30% en poids au moins.

6. Tissu de type non tissé selon la revendication 1, dans lequel la composition des stabilisateurs UV est présente à hauteur de 0,5 à 5% en poids par rapport au tissu microfibreux de type non tissé.

7. Tissu de type non tissé selon la revendication 6, dans lequel la composition des stabilisateurs UV est présente à hauteur de 1,5 à 3% en poids par rapport au tissu microfibreux de type non tissé.

8. Tissu de type non tissé selon la revendication 3, dans lequel le polyester est un polyéthylène-téréphtalate.

9. Tissu de type non tissé selon la revendication 3, dans lequel le polyester consiste en un mélange de polyéthylène-téréphtalate et de polyéthylène-téréphtalate colorable avec des colorants cationiques.

10. Procédé de fabrication du tissu microfibreux chamois de type non tissé de la revendication 1, le procédé comprenant :
préparation d'un tissu microfibreux chamois écru de type non tissé ;
coloration du tissu microfibreux chamois écru de type non tissé pour obtenir un produit coloré ;
et
traitement du produit coloré avec une composition de stabilisateurs UV consistant en :
au moins une triazine ou ses dérivés, ayant une absorption maximale à des longueurs d'onde allant de 270 à 285 nm ; et
au moins un composé sélectionné à partir de benzophénones, de benzotriazoles, et des mélanges de ceux-ci.

11. Procédé selon la revendication 10, dans lequel les étapes de coloration et de traitement sont effectuées en même temps.
